

# United States Patent Office.

A. G. HUNTER, OF FLINT, WALES.

*Letters Patent No. 77,618, dated May 5, 1868.*

## IMPROVEMENT IN THE MANUFACTURE OF ZINC.

The Schedule referred to in these Letters Patent and making part of the same.

TO ALL WHOM IT MAY CONCERN:

Be it known that I, A. G. HUNTER, of Flint, Wales, temporarily residing in Fair Haven, in the county of New Haven, and State of Connecticut, have invented a new Improvement in the Manufacture of Zinc; and I do hereby declare the following to be a full, clear, and exact description of the same.

In the ordinary process of smelting zinc, the ore, after suitable preliminary treatment, is intimately mixed with carbonaceous matter, the mixture then placed in retorts or crucibles, and the zinc distilled off by a high heat. Great expense and loss are incurred by the use of such retorts or crucibles, and my improvement relates to a process whereby their use is dispensed with.

In order to the clear understanding of my improvement, I will proceed to a full description of the same.

I take the zinc ores, after having been subjected to the usual preliminary treatment, and intimately mix them with the usual quantity of carbonaceous matter, and place this mixture on the hearth of a reverberatory furnace, in which it is acted on directly by the heat and flame from the fire. In order to effect the reduction of the zinc from its ore, care must be taken to prevent the presence of any free oxygen in the flame, or heated gases passing over the zinc-ore mixture. This may be accomplished either by keeping a thick mass of burning fuel in the fireplace, or by introducing carbonic oxide, carburets of hydrogen, or hydrogen gas, or other deoxidizing agent, at the fire-bridge, so as to be mixed with the flame from the fire before it reaches the zinc-ore mixture, care being taken to prevent the admission of air at any other part of the furnace except through the grate-bars of the fireplace, which must be well filled with fuel while the zinc-ore mixture is under treatment. By the reducing-action of the heated gases and flame, and of the carbonaceous matter mixed with the ore, the zinc the ore contains is liberated in a metallic state, and distills off as a vapor, mixed with the heated gases and flame from the fire. I condense the zinc vapor to metal by causing the heated gases, flame, and zinc vapor, previous to their reaching the chimney, to pass through a pipe or condenser surrounded with water, which cools the gases sufficiently to allow the zinc to deposit in a metallic state. I provide, in this pipe or condenser, suitable recesses or cess-pools, to receive the melted zinc as deposited, from which it may be run off into moulds; also suitable openings, through which the pipe may be cleaned out. Either a stationary or a revolving reverberatory furnace may be used to heat the zinc ores in, and the condenser may be either vertical or horizontal, or both alternately, and the sizes of the furnace and condenser may be varied, to suit the amount of work required to be done. I have found a furnace-hearth eight feet square, and a condenser twenty inches diameter and sixty feet long, a convenient size; but these proportions may be varied.

Having thus fully described my invention, what I claim as new and useful, and desire to secure by Letters Patent, is—

The process of extracting zinc from its ores by the direct application of heat to the said ores, without the use of crucibles or retorts to contain the said ores, the heated gases and flame being, previously to their contact with the zinc, carefully deprived of free oxygen, and the subsequent condensation of the zinc vapor to the metallic state, all substantially as herein described.

A. G. HUNTER.

Witnesses:

A. J. TIBBITS,  
J. H. SHUMWAY.